

Dec. 7, 1948.

G. H. BENDIX

2,455,726

METHOD FOR ELECTROLYTIC STRIPPING AND  
DETERMINATION OF PLATING METAL  
Filed July 13, 1942

FIG. 1.



FIG. 2.



Inventor

Gordon H. Bendix,

By

Mason, Porter & Dillen,

Attorneys

## UNITED STATES PATENT OFFICE

2,455,726

## METHOD FOR ELECTROLYTIC STRIPPING AND DETERMINATION OF PLATING METAL

Gordon H. Bendix, Chicago, Ill., assignor to Continental Can Company, Inc., New York, N. Y., a corporation of New York

Application July 13, 1942, Serial No. 450,750

4 Claims. (Cl. 204—1)

1

This invention relates to the stripping of multi-valent plating metal from material, and is particularly concerned with such stripping as means of determining the amount of plating metal which is present in the plated material.

It has heretofore been proposed to employ electrolytic stripping for removing the plating metal through an oxidizing operation, with the utilization of an electrolyte of oxidizing character, followed by a determination of the decrease of oxidizing power of the body of the electrolyte; but such prior proposals have been coupled with the difficulty that these determinations were not exact and it was necessary to make allowance for certain phases of treatment by employment of standard times, allowances for the size and operation of the apparatus, etc.

A feature of the present invention is the provision of apparatus and method by which such determinations can be effected without close manual control and visual observation of the course of the stripping.

Another feature of the invention is the provision of an apparatus and method by which the determination can be effected upon the entirety of standardized specimens of plated sheets, in a simple and convenient manner.

A further feature of the invention is the provision of an apparatus and method by which plated metal, having coatings on both sides, may be subjected to a single operation for determining the amount of plating metal present, without requirement of comparison tests against blanks, and without requiring a standard time of operation.

With these and other features as objects in view, an illustrative form of practicing the invention is set out in the following description, in association with the drawings, in which:

Figure 1 is an upright sectional view through an electrolytic stripping apparatus, comprising a container and stand and the associated structures for performing the process, being taken substantially on line 1—1 of Fig. 2.

Figure 2 is a sectional view of the container with its associated parts, taken substantially on line 2—2 of Fig. 1.

In these drawings and the detailed description thereof is set out a preferred form of employing the invention in determining the weight or

2

thickness of the tin coating in a normal tin plate. For this purpose, a specimen is prepared which has a definite area, and is made the anode between two carbon cathodes which are shut off from the anode by diaphragm means. In practice, a round specimen 2.418 inches in diameter (4 square inches area, one side) is a desirable form. Surrounding the specimen is an anolyte comprising a solution of iodine and potassium iodide in dilute hydrochloric acid. The catholyte in this preferred form of practice is dilute hydrochloric acid. Upon passage of a direct current at a current density of about three amperes (i. e. three-eighths ampere per square inch, for the two sides), for about two minutes, the tin is stripped from a specimen of the tin plate as employed for forming food containers, this tin passing initially into the solution in the stannous state. During this stripping of the tin, a chemically equivalent amount of hydrogen ions is discharged at the cathodes and passes off into the atmosphere without coming into contact with the iodine solution. Secondarily, the iodine in the anolyte reacts with the stannous tin to oxidize it to the stannic state, and is itself reduced to iodide. The quantity of iodine thus converted to iodide is directly proportional to the quantity of tin dissolved, and hence a determination of the decrease of elemental iodine content from the beginning of the electrolysis to the end of the electrolysis permits computation of the amount of tin which has been stripped from the tin plate.

It has been found in practice that no significant interfering reactions occur at the anode or in the anolyte, and that the segregation of the catholyte, so that cathode hydrogen is prevented from contact with the anolyte or with the anode, permits direct determinations rapidly and accurately.

40 In the apparatus shown on the drawings, a stand 10 has a narrow elevated ledge 11, a projecting finger 12, and a shelf 13. A container B, such as the 400 millimeter glass beaker of standard type, may be introduced to the stand 45 by engaging its lip with the finger 12 and then rocking the beaker into position so that it can rest on ledge 11.

The shelf 13 is apertured to receive and support the two porous cups 15 having the enlarged flanges 16, the cups 15 being within the con-

tainer B when the latter is mounted on the stand. A metal support 17 is secured to the back wall of the stand 10 and has a vertical aperture through which may be slid the iron pole piece 18, which passes through a small aperture in the shelf 13 and thus into the container B at a point between the two porous cups 15. The porous cups 15 receive the stoppers 19, which may be of glass and in which are mounted carbon rods 20 constituting cathodes which are thus positioned within the cathode compartments formed by the porous cups 15.

A conductor 21 is connected to the two cathodes 20 and extends to the negative terminal of a source 22 of direct current, and a conductor 23 extends from the source 22 and is connected, in this preferred form, to the support 17. The current flowing may be read by an ammeter A included in one of these conductors. A branch 24 from the conductor 23 includes a rheostat 25 and supplies current to the winding 26 which is positioned around the pole piece 18, with a current return by conductor 27 to conductor 21.

The determinations are effected by preparing a specimen S which is illustrated as being a disc cut from the material to be tested. The pole piece 18 may be adjusted vertically and secured by the screw 17a so that its lower end is at or slightly below the standard liquid level in the container B. The current from the battery 22 flows by the conductors and winding 26 so that the pole piece 18 is magnetized, and is thus capable of supporting the specimen S by its edge in totally submerged conduction in the standard volume of solution in the container B.

During the course of testing, the lower end of the pole piece 18 may be eaten away, but it is then a simple matter to relieve the screw 17a, and adjust the pole piece downwardly.

The container is provided with a standard quantity of reagent solution, and then is introduced into the stand, so that the liquid level is above the top of the specimen S. The flow of current through the conductors 21, 23 causes electrolysis within the cell so that the aforementioned reactions occur therein.

Preliminary to the determinations, certain reagents are prepared as stock solutions. The concentrations relative to iodine should be between 0.2 and 0.01 normal. At the higher end of this range, accurate titration becomes difficult; and at the lower end, the starch end point is sometimes indistinct. Examples of good practice for the reagents are:

A N/10 normal potassium iodate solution is prepared by dissolving 3.566 grams of potassium iodate, 22 grams of potassium iodide, and 1 gram of sodium hydroxide in water made up to a volume of 1 liter. The alkali serves to prevent hydrolysis of the iodate. This solution must be made up accurately with respect to the weight of potassium iodate per volume, or as an alternative it may be standardized upon titration against a suitable standard such as arsenic trioxide.

A N/10 normal solution of sodium thiosulfate is prepared by dissolving 25 grams of crystalline sodium thiosulfate ( $\text{Na}_2\text{S}_2\text{O}_3 \cdot 5\text{H}_2\text{O}$ ) with 0.1 gram of sodium carbonate in water to make up 1 liter. This solution is about N/10, and is then standardized against the N/10 potassium iodate solution above.

A dilute hydrochloric acid solution is prepared by diluting concentrated (1.19 sp. gr.) hydrochloric acid with four to ten times its volume of water: the present preference is a ratio of 1:7.

A starch indicator of 0.2 percent strength is prepared by dissolving 2 grams of soluble starch in 1 liter of boiling water, and cooling. A trace of a preservative such as chloroform or mercuric iodide may be added.

These solutions will keep for a considerable period of time, and need not be freshly prepared immediately prior to use.

In preparing for tests, dilute hydrochloric acid is introduced into the porous cups, and a body of anolyte is placed in the container 14. This anolyte is prepared by introducing approximately 200 milliliters of dilute hydrochloric acid into a 400 milliliter beaker and adding an accurately measured quantity of 20 milliliters of the N/10 normal potassium iodate solution. A reaction then occurs:



The quantities employed assure an excess of hydrochloric acid, and hence no iodate is present in this anolyte, and by thus freshly preparing the same, its content of iodine is standardized.

The material to be tested, in this illustration being a sheet of tin plate, is then cut, preferably by a standard punch, to provide a disk 25 of standard area. The tin plate is comprised of the base black plate of ferrous material with a coating of tin on each side thereof. This specimen is brought against the pole piece of the magnet 18 and is suspended thereby. It will be noted that it thus acts as an armature, but only makes contact at limited portions and at its periphery, so that the tin plating is fully exposed to the anolyte.

The beaker with its content of anolyte is then raised into position and brought to rest on the ledge 11.

Current is then allowed to flow at a rate of about 3 amperes for a specimen having a standard area of 4 square inches, for a time of about 2 minutes with tin plate as employed for food containers. The amperage and time may be varied within fairly wide limits but care, on the one hand, should be taken that sufficient current

passes to dissolve all of the tin from the sample. With this preferred practice, about 1 minute is required for stripping the tin, and an extra minute is allowed for safety. On the other hand, the cell should not be operated longer than about 5 minutes with the above solution and at 3 amperes intensity, as otherwise excessive dissolution of iron occurs and slightly high results may be obtained. For the illustrated example, therefore, a time of 1 to 5 minutes may be employed, without essential change in the accuracy of the result.

While the current is flowing, the tin at the anode becomes electrically charged and passes into the solution:



At the anode, after the tin has been dissolved, a reaction occurs:



At the cathode, hydrogen ions are discharged and hydrogen gas is formed:



The stannous tin ions formed at the anode by Reaction 2 are oxidized by the iodine according to the following reaction:



No significant reaction occurs between the iodine and the ferrous ions formed by Reaction 3, unless the cell is operated for an excessively long time (6 minutes or more for the above conditions), or at an excessively high current density. 5

The electrolytic operation removes the tin plating and also any tin which is present in the form of a tin-iron alloy.

The beaker and its contents are now removed, and titration is accomplished with N/10 sodium thiosulfate solution which is added slowly from a burette until the iodine solution has only a light straw color. A few milliliters of starch indicator solution are stirred in, and the addition of sodium thiosulfate is continued until the solution changes 15 color from blue to water white upon the addition of a single drop.

The amount of tin can then be computed from the volume of sodium thiosulfate required for the reduction of the iodine solution, as the decrease 20 of oxidizing power of the iodine solution is directly related to the quantity of tin which has been oxidized from stannous to stannic condition.

As an example of such computation, with a piece of tin plate having an area of 4 square inches (one side), the potassium iodide solution contains 3.442 grams of  $KIO_3$  per liter and has an oxidation normality (molecular weight of  $KIO_3=214.0$ ) of  $(3.442 \times 6) / 214.0 = 0.0965$  N (or about N/10).

Upon control analysis of a standard amount, such as employed above in the breaker 14, it is found that the 20 milliliters of  $KIO_3$  solution requires 21.1 milliliters of standard sodium thiosulfate solution, before electrolysis; so that 1 milliliter of sodium thiosulfate solution is equivalent to 0.948 milliliter of  $KIO_3$  solution.

With the particular specimen, for assumption, 2.47 milliliters of  $Na_2S_2O_3$  solution was required for titrating the iodine after electrolysis of the specimen. Therefore,  $21.10 - 2.47 = 18.63$  milliliter of  $Na_2S_2O_3$  solution represents the change by reason of employment of iodine for oxidizing the stannous tin. This quantity is equivalent to  $18.63 \times 0.948 = 17.66$  milliliters of  $KIO_3$  solution. Since this solution was 0.0965 N, and was effective to increase the valency of the tin by 2 electrons per molecule, it can then be computed:

$$17.66 \times 0.0965 \times \frac{118.7}{2} = 101.2 \text{ mg. of tin}$$

where 118.7 is the atomic weight of tin.

This specimen of tin (4 square inches) with its coating of 101.2 milligrams of tin corresponds to 1.75 pounds of tin per base box, which is the standard of quantity in computing the weight of tin coating commercially.

This computation need not be made each time, but a table can be constructed in which the weight of tin per base box is indicated as a direct function of the volume of sodium thiosulfate required for reducing the remaining iodine after the electrolysis.

The invention therefore provides a simple and convenient apparatus and method for the quick determination of the weight of tin coatings.

While the invention has been described in detail in an application to evaluating the weight and thickness of tin coatings upon tin plate, it will be understood that it can be employed more generally to the evaluation of multivalent plating metals, such as tin, upon ferrous and other bases, with employment of proper stripping electrolysis.

by utilization of the step of preventing the action of cathode hydrogen upon the electrolyte, by which the exactness of determination of the decreased oxidizing power of the electrolyte would otherwise be obscured.

I claim:

1. The method of determining the amount of tin present in tin plate having a ferrous base, which comprises magnetically suspending a specimen of the tin plate by its edge in an anolyte containing a standard quantity of elemental iodine in the presence of hydrochloric acid, passing electric current with said specimen as anode and employing a separate catholyte for preventing contact of the cathode hydrogen with the electrolyte, and determining the amount of iodine consumed during the stripping as the direct indication of the amount of tin originally present on the tin plate.

2. The method of determining the amount of tin present in tin plate having a ferrous base, which comprises magnetically suspending a specimen of the tin plate by its edge in a standard quantity of anolyte prepared by mixing a solution substantially deci-normal in potassium iodate and containing substantially 22 grams of potassium iodide per liter with a solution containing concentrated hydrochloric acid to the amount of 180 milliliters of acid per liter of anolyte, said mixed solutions containing hydrochloric acid beyond the quantity for reaction with the iodate, passing electric current with said specimen as anode and at a current density of substantially  $\frac{3}{8}$  ampere per square inch of total specimen area for a time of substantially 2 to 6 minutes and until all the tin and essentially no base metal has entered the anolyte, with the employment of a cathode within the separated catholyte whereby to prevent contact of the cathode hydrogen with the anolyte, and determining the amount of iodine consumed during the stripping as the direct indication of the amount of tin originally present on the tin plate.

3. The method of determining the amount of tin present in tin plate having a ferrous base, which comprises magnetically suspending a specimen of the tin plate by its edge between two catholyte chambers and in an anolyte mechanically separated from mixture with the catholyte, said chambers being individually located opposite the faces of the tin plate specimen, said anolyte comprising a standard quantity of iodine and containing potassium halide and hydrochloric acid, the catholyte chambers being effective to prevent contact of the cathode hydrogen with the anolyte, passing electric current with said specimen as anode, and determining the amount of iodine consumed during the stripping as the direct indication of the amount of tin originally present on the tin plate.

4. The method of determining the amount of tin present in tin plate having a ferrous base, which comprises magnetically suspending a specimen of the tin plate by its edge, electrolytically stripping the tin from the tin plate specimen as anode in a hydrochloric acid solution containing a known quantity of iodine and potassium iodide and in the absence of potassium iodate, and with a separated catholyte for preventing contact of the cathode hydrogen with said solution; removing the solution after all the plating metal has been stripped and prior to essential removal of the base metal of the tin plate; and determining the amount of iodine consumed during the stripping

as the direct indication of the amount of tin originally present on the tin plate.

GORDON H. BENDIX.

#### REFERENCES CITED

The following references are of record in the file of this patent:

#### UNITED STATES PATENTS

| Number    | Name      | Date          |
|-----------|-----------|---------------|
| 442,333   | Roberts   | Dec. 9, 1890  |
| 1,168,280 | Buch      | Jan. 18, 1916 |
| 1,235,202 | Hartsuch  | July 31, 1917 |
| 1,287,156 | Whitehead | Dec. 10, 1918 |
| 1,724,928 | Hailwood  | Aug. 20, 1929 |

10

5

7

8

#### FOREIGN PATENTS

| Number  | Country       | Date         |
|---------|---------------|--------------|
| 485,089 | Great Britain | May 13, 1938 |

#### OTHER REFERENCES

Treatise on Inorganic and Theoretical Chemistry, vol. II (1922), page 315.

Journal of the Electrodepositors' Technical Society, vol. XI (1935-36), pp. 16, 17, 20.